# EUROPEAN PATENT APPLICATION

(11) **EP 1 867 781 A1**
(43) Date of publication of application: **19.12.2007**
(21) Application number: 05850521.5
(22) Date of filing: 14.03.2005
(51) Int. Cl.: D06Q 1/08, D06P 7/00, D06C 23/04

(54) **DECORATION OF EMBOSSED TEXTILES**

(71) Applicant: Piel, S.A., 46890 Agullent (Valencia) (ES)
(72) Inventor: MULLOR VIDAL, Joaquin, E-46870 Ontinyent (ES)
(74) Representative: Chanza Jordan, Dionisio
(86) International application number: PCT/ES2005/070026
(87) International publication number: WO 2006/100322

(57) **Abstract**

The invention relates to the decoration of embossed textiles, which enables the use of macromolecular substances on thick textile pieces comprising synthetic or natural long pile in order to counteract deterioration caused by normal use or successive washing operations, conferring thereon gold and silver aesthetic effects. The textile treatment method consists in first embossing or thermoengraving a corresponding pattern disposed in an embossing mould on a thick textile piece with natural or synthetic pile. Subsequently, the embossing mould in the embossing machine is replaced with a stamping mould having an identical pattern, which stamps and prints a layer of the selected macromolecular substance, purpurin or polyester particles. The product is then applied uniformly by means of scraping using either a rod or a scraper. Finally, the folds are dried with thermal air in the same machine in order to polymerise and set the stamped product.

## Description

The invention relates to the decoration of embossed textiles which enables the use of macromolecular substances on thick textile pieces.

It is therefore, a local decoration process that allows configuring ornaments with multiple patterns, based on the priming of macromolecular substances, mainly metallic powder - mineral powder - and frosts - polyester powder - onto the fabrics to be decorated; this produces an optical effect of highlighting the embossed patterns in a relief.

The use of embossed ornaments on textiles also known as heat-etched is a well known and usual activity in the fabrics manufacture and sale industry. However, the inclusion of metallic powder on textile products was not possible, resulting in the lack of consistency and adherence for future washes and long lasting usage. This invention achieves a fixing treatment and therefore greater durability to the printed substances.

Today, chemical compositions are applied directly without embossing to decorate fabrics - mainly powder of various colours and polyester particles; however because these are adhered only with glue or synthetic resins, their resistance and durability is limited under regular use or cleaning and washing of fabrics. In addition, the so-called natural or synthetic pile products (for example blankets and carpets), the inclusion of macromolecular substances to provide ornamental effects has not been developed for industrial and commercial purposes, considering the flexibility and fragility of pile fibres; the ornamental effects are performed either by combinations of various pieces joined together or by printings of different patterns and colours.

In summary, the described invention provides a technical advantage such as provide stability to the printed substance and permanent shine and luminosity, providing resistance to subsequent washes or against deterioration from normal and regular usage over time. It also produces an aesthetic advantage such as the possibility of producing multiple patterns and colours using fabrics with metallic powder and polyester flakes, specifically, on pile items.

Finally, it results in novel commercial applications for the home textile market, as it is possible to sell products with purpurin or metallic powder and polyester particles maintaining their stability and resistance on textiles.

Today, there are several fabric decoration procedures and treatments that are known and used, but they all present different operational and functional purposes, especially for not being applied in the goffer or heat-etching fields or provided stability and durability qualities to the printed substances; therefore the use of already development means involve several limitations compared to this invention, based on its technical and financial advantages. Hence, there are several fabric decoration solutions such as the procedure for printing on fabrics with a mixture of cellulose and polyester defined in the Spanish Patent number 0477136, or a procedure to obtain fabrics with a pearly finish defined in the Spanish Patent number 0433728, or also the method to obtain fantasy chromatic finishes on fabrics defined in the Spanish Patent 0387798, or the North American invention patent number US1510250, to achieve opalescent and fluorescent effects on fabrics; all of these prior inventions similar to the invention being presented, but generic and inaccurate and as inventions that result average or not specific to embossed fabrics, or not developed with the same or equivalent treatment phases in the textile decoration process.

These textiles procedures and treatments are different to the invention defined herein, which can be executed and produced as follows:
First, using a thick fabric or of natural or synthetic pile, the pattern is printed onto the embossing mould; the result is a relief on the fabric that shortens the length of the pile and flattens the drawn surface. Next, the embossing mould is replaced on the embossing machine with a pattern mould equal to the drawing, which stamps and prints a layer of the selected macromolecular substance - metallic powder or polyester flakes, mainly - depending on the chosen colour pigments. Next, the product is applied uniformly using a rod-based scraping procedure. And finally, the same machine dries the folds to polymerize and fix the stamped product, providing the final consistency.

With regards to the chemical components, the macromolecular substance used is combined and based on a bonding and adherent resin, mixed with a colour pigment.

In summary, with the product resulting from the progressive and gradual treatment results in an aesthetic advantage by printing bright macromolecular substances with golden and silver effects on embossed patterns. This also produces a technical advantage that is a product of greater stability and resistance to usage on fabric and its subsequent cleaning, as the substance applied sets on a flat pattern surface over the entire embossed pattern and not on fibres or long piles, which are flexible materials in terms of grouped filaments.

## Claims

1. Decoration of embossed textiles **characterized by** a textile treatment method by embossing or thermoengraving a corresponding pattern disposed in an embossing mould on a thick textile piece with natural or synthetic pile. Subsequently, the embossing mould in the embossing machine is replaced with a stamping mould having an identical pattern, which stamps and prints a layer of the selected macromolecular substance, purpurin or polyester particles. The product is then applied uniformly by means of scraping using either a rod or a scraper. Finally, the folds are dried with thermal air in the same machine in order to polymerise and set the stamped product.

2. - Decoration of embossed textiles according to Claim 1, **characterized** because it provides a macromolecular substance based on purpurin or metal powder particles combined with a bonding and adherent resin, mixed with a colour pigment.

3. - Decoration of embossed textiles according to Claim 1, **characterized** because it provides a macromolecular substance based on polyester particles combined with a bonding and adherent resin, mixed with a colour pigment.
